

Patented Feb. 27, 1934

1,949,112

# UNITED STATES PATENT OFFICE

1,949,112

## RIVETED PLATED ALUMINIUM ARTICLE

Gustav Schreiber, Bitterfeld, Germany, assignor  
to I. G. Farbenindustrie Aktiengesellschaft,  
Frankfort-on-the-Main, Germany

No Drawing. Application July 8, 1931, Serial  
No. 549,574. In Germany July 18, 1930

4 Claims. (Cl. 29—181)

The present invention relates to improvements in the riveting of plated aluminium articles and is more especially concerned with an improved rivet to be employed for this purpose with advantageous results in respect of the mechanical strength and the resistance to corrosion of such articles.

It is well known that certain aluminium alloys having a high mechanical resistance, particularly alloys belonging to the duralumin type, have a very limited resistance to the action of sea-water and similar corroding agents. In order to overcome this deficiency it has been proposed to provide articles made of such high strength aluminium alloys with a skin or plating of a metal having a high resistance to corrosion, particularly technically pure aluminium. Thus, an article combining a high mechanical strength with a surface which is particularly resistant to corrosion is obtained. The method in question has been widely employed for the manufacture of light metal sheets, and products obtained in this manner have become known under the names of "Alclad" or "Alplat".

Insofar as a riveting of such articles is required, this was hitherto generally effected by means of duralumin rivets, so as to ensure high mechanical strength also in the combination. However, it has transpired that the vicinity of such rivets is liable to particularly violent corrosion, due to the relatively large electrolytic potential difference between the rivet material and the plating metal. On the other hand, the employment of rivets of pure aluminium, which recommends it self from the point of view of smallest possible difference in electrolytic potential as compared with that of the plating metal, is impracticable owing to the inferior mechanical strength properties of the pure metal. Accordingly, the present invention provides for a rivet material having at the same time a high strength and an electrolytic potential remaining approximately equal to that of the coating metal, namely technically pure aluminium.

I have ascertained that alloys containing between about 4 and 7 percent of magnesium, re-

mainder aluminium, have a mechanical strength which is entirely sufficient to resist the stresses to which rivets are subjected, and at the same time do not give rise to any perceptible corrosion in contact with pure aluminium. Thus, rivets made from these alloys fulfill the object of the present invention.

The mechanical strength of the alloys to be employed for making rivets according to the present invention can be further improved by incorporating therein a small quantity of manganese (between about .3 and 1 percent).

Whenever technically pure aluminium is mentioned as the metal constituting the plating of the articles, it is to be understood that this term, in the sense of the invention, also comprises any alloy or metal having substantially the same electrolytic potential as technically pure aluminium itself.

I claim:

1. A structure comprising sheets of a high strength aluminium alloy coated with technically pure aluminium and rivets joining such sheets, the rivets being composed of a high grade aluminium alloy containing between about 4 and 7% of magnesium and having an electrolytic potential remaining approximately equal to that of technically pure aluminium.

2. A structure comprising sheets of a high strength aluminium alloy coated with technically pure aluminium and rivets joining such sheets, the rivets being composed of an alloy of between about 4 and 7% of magnesium, the balance being aluminium.

3. A structure comprising sheets of a duralumin alloy coated with technically pure aluminium and rivets joining such sheets, the rivets being composed of an alloy of between about 4 and 7% of magnesium, the balance being aluminium.

4. The structure defined in claim 2 wherein the alloy of the rivets contains between about 4 and 7% of magnesium and about .3 and 1% of manganese, the balance being aluminium.

100

GUSTAV SCHREIBER.

105